

May 12, 1931.

F. W. HAMMOND

1,805,215

MEANS FOR COATING METALLIC ARTICLES, PARTICULARLY  
THE INTERIORS OF WATER MAINS (IN SITU)

Filed May 13, 1930

2 Sheets-Sheet 1

*Fig. 1.*



*Fig. 2.*



*Fig. 3.*



*Fig. 4.*



*Fig. 5.*



INVENTOR  
FREDERICK W. HAMMOND

By D. P. Wachanoff Atty.

May 12, 1931.

F. W. HAMMOND

1,805,215

MEANS FOR COATING METALLIC ARTICLES, PARTICULARLY  
THE INTERIORS OF WATER MAINS (IN SITU)

Filed May 13, 1930

2 Sheets-Sheet 2

Fig. 6.



Fig. 7.



INVENTOR  
FREDERICK W. HAMMOND

By D. P. Welch, Atty

## UNITED STATES PATENT OFFICE

FREDERICK WILLIAM HAMMOND, OF CHEPSTOW, ENGLAND

## MEANS FOR COATING METALLIC ARTICLES, PARTICULARLY THE INTERIORS OF WATER MAINS (IN SITU)

Application filed May 13, 1930, Serial No. 452,116, and in Great Britain March 5, 1930.

This invention provides improved means for depositing a protective coating on metallic articles, particularly the interior surfaces of water mains (in situ) including a 5 colloidal solution or emulsion of fluxed bitumen and other ingredients in an aqueous medium from which the said coating is deposited by electrolysis between an anode consisting of the positively charged metallic 10 article to be coated and a negatively charged cathode which is movable opposite to and along the surfaces of said metallic articles, and a source of direct electric current.

It has been found in practice that after 15 scraping and clearing away the deposits of organic and inorganic grounds in water mains, fresh deposits set up very quickly, due to inferior pipes or pipes with inferior bituminous coating and to the action of the 20 water conveyed, with the result that objectionable discoloured water is supplied and an important object of this invention is to prevent such re-growth of deposits and discolouration of the water.

25 The present invention therefore provides a protective solution or emulsion containing fluxed bitumen and other ingredients and apparatus whereby the said solution or emulsion is deposited by electrolysis on the surfaces of the metallic articles so as to leave a smooth and coherent continuous coating, 30 impervious to water, of colloidal particles of bitumen with other protective ingredients.

The electrolytic coating is deposited from 35 a colloidal solution or emulsion which includes pure petroleum bitumen fluxed with asphalt oil and/or paraffin wax, with or without a percentage of saponaceous material plus a protective adhesive colloid such 40 as casein, gum or strach as emulgant.

In certain cases the electrolytic solution 45 may include pure petroleum bitumen fluxed with asphalt oil and have a percentage of casein, gum or strach, or in addition to the foregoing ingredients the solution may contain a percentage of saponaceous material.

In other cases the electrolyte may include 50 pure petroleum bitumen fluxed with asphalt oil and paraffin wax of either one of these fluxes and have a percentage of casein, gum

or strach as adhesive and emulgant, or in addition to the aforesaid ingredients there may be saponaceous material such as alkali and fatty acid.

The fluxed bitumen content of the electrolytic solution is approximately 25% of the total weight of the solution, and of the other ingredients when included, from 0.25% to 0.5% of alkali, from 0.25% to 0.5% of fatty acid, from 0.05% to 0.1% of casein, gum or strach.

The electrolyte is applied by partial or total immersion or by spraying, to the article to be coated which is connected as one of the electrodes to one pole of a dynamo while the other electrode, which is of shape or section conforming suitably to that of the articles to be coated, contains or is immersed in the electrolyte and is connected to the other pole of the dynamo.

The article to be coated is connected to the positive pole of the dynamo as anode, and the shaped electrode to the negative pole as cathode, the latter, when water pipes are to be coated, being a metallic tube or cylinder mounted on a carriage of insulating material and caused to travel through the water pipes which are first filled with the electrolyte, or the latter may alternately be sprayed in jets from the negatively charged cathode as it travels through the water pipes or a cathode sealed at each end by hydraulic washers and carrying its own supply of electrolyte fed by a hosepipe as it travels or is drawn through the water pipes, may be used.

In order that the invention may be clearly understood, there will now be described with the aid of the accompanying drawings, various modifications of the apparatus suitable for metal articles of different kinds and sizes.

In the drawings:—

Figure 1 is a diagram showing the application of the process to metal articles generally.

Figures 2 and 3 are longitudinal and cross sections respectively of a water pipe of small diameter, to be filled with the electrolyte and with suitable apparatus therein.

Figures 4 and 5 are longitudinal and cross

sections respectively of a water pipe too large to be filled with electrolyte and fitted with apparatus carrying its own supply of electrolyte.

5 Figures 6 and 7 are longitudinal and cross sections respectively of a very large water main with apparatus suitable for localized application of the electrolyte.

Referring first to Figure 1, which shows 10 the application to metallic articles generally which are of moderate size and compact shape, a suitable vessel 1 contains the electrolytic solution, the article 2 which is to be coated and which is connected to the positive 15 pole 3 of the electric supply, and also the negatively charged cathode 4 which is connected to the negative pole 5. The cathode 4 may be moved opposite to and along the surfaces of the article 2 when the latter is of 20 sufficient area or extent to require such movement. A voltmeter 6 and ammeter 7 are provided in the circuit in order that the electric supply may be regulated through the electrolyte.

25 For water pipes of small or moderate diameter, as shown in Figures 2 and 3, the pipe 8 is to be filled with the electrolyte from a tank or by other suitable means, and into the pipe 8 there is introduced a cylinder 9 preferably of copper as the negatively charged cathode which is arranged to be drawn through the pipe 8 by a cord or wire rope fixed to an insulating bridge-piece 10. A carriage 11 of insulating material, such as 30 hardwood, supports the cylinder 9 and is fitted with rubber discs or rings 12 to centre the cylinder 9 in the pipe 8 and to facilitate its passage therethrough. The rings 12 are 35 perforated or have scalloped edges to allow 40 free passage of the cathode 9 through the electrolyte, but the rings are staggered so that the perforations are not in direct alignment to prevent the pipe 8 being coated imperfectly ahead of the cathode 9. Four of 45 the rings 12 are generally employed but these may be added to with advantage for larger pipes.

Waterproof cable 13 is connected to a terminal 14 on the front end of the carriage 11 50 and a central conductor 15 connects between the terminal 14 and the cylinder 9 via a flexible lead 16. There is a wooden boss 17 at the rear of the cylinder 9 to prevent it from 55 touching the walls of the pipe 8 and so making a short-circuit for the current.

Referring now to Figures 4 and 5, the cathode 18 is for use with pipes which are 60 too large to be easily filled with electrolyte and it has at the ends carriages 19 and 20 of insulating material, such as hardwood, which are fitted with rubber discs or rings 21 and leather hydraulic washers 22 which centre and insulate the cathode 18 in the water 65 pipe 23 and also seal a supply of electrolyte

which is carried between the cathode 18 and the water pipe 23.

The electrolyte is fed through a hosepipe 24 to a tube 25 running through the front carriage 19 and emerging through the surface 70 of the cathode cylinder 18, any surplus being allowed to escape past the rear rubber ring 21 and hydraulic washer 22. This is necessary to maintain the concentration of bitumen required in the electrolyte in use 75 between the cathode cylinder 18 and the water pipe 23.

The numbers of rubber rings and hydraulic washers used depend on the size of the water pipe to be coated, being one or more of each 80 per carriage.

Means of supplying electric current and means of hauling through the water pipe are provided as hereinbefore described and the cathodes are in all cases to be drawn through 85 their respective pipes at such a speed as will ensure correct deposition of the bitumen particles.

Referring now to Figures 6 and 7, which 90 illustrate an apparatus for coating pipes large enough to admit of the ingress of a man, the cathode is a brass plate 26 curved to the shape of the inner surface of the water pipe 27 and is held in a box 28 of insulating material, such as hardwood, similarly curved 95 to the pipe 27; the cathode plate 26 is insulated from the pipe 27 by a flexible rubber edging 29 which also serves as a seal for the electrolyte between the pipe 27 and the cathode plate 26.

A supply tube 30 is articulated to the box 28 and conveys a supply of electrolyte from a suitable reservoir to the box 28 and to the space between the cathode plate 26 and the inner surface of the water pipe 27 via a hosepipe 31 and a short tube 32 emerging through the surface of the cathode plate 26; a valve 33 is provided at the top end of the tube 30 to control the flow of the electrolyte. The tube 30 is universally jointed by being held by a ball 34 between two cups 35 and 36 midway between two wood-wheeled trolleys 37 and 38 forming a travelling carriage and being held against the top and bottom of the pipe 27 by two telescopic screwed struts 39 and 40 capable of being extended or contracted by two hand nuts 41 and 42, enabling the apparatus to be adjusted to the diameter of the pipe.

Electric current is provided and is supplied 120 to the cathode plate 26 by the waterproof cable 43 connected to said plate 26 through box 28 and is controlled by the ammeter 44 and switch 45.

A third telescopic screwed strut 46 behind the top end of tube 30 and the water pipe 27 and controlled by the hand nut 47 and fitted with a friction pad 48, enables the cathode plate and box 28 to be firmly held against any desired portion of the interior surface 130

of the water pipe 27, the ball 34 and cups 35 and 36 controlling radial movement and the trolleys 37 and 38 controlling longitudinal movement in the pipe 27.

The pipe 27 can be coated at any desired part by straining the box 28 to the interior surface of the pipe 27, flooding the space between the cathode plate 26 and the pipe 27 and switching on the electric current for such a period of time as will ensure correct deposition of the bitumen particles.

The electric supply may be from a portable dynamo or from public supply mains giving direct current at about 100 to 110 volts whilst the current starts at about 0.16 amperes per square inch of surface to be coated and falls to a lower figure as the surface becomes coated.

I claim:—

1. Improved means for depositing a protective coating on metallic articles, including a colloidal solution or emulsion or fluxed bitumen and other ingredients in an aqueous medium from which said coating is deposited by electrolysis, an anode consisting of the positively charged water pipe to be coated, a cathode consisting of a negatively charged copper cylinder movable through said water pipe by a rope attached to a bridge-piece on said cylinder, a travelling carriage of insulating material supporting said cylinder and fitted with rubber discs or rings, a waterproof cable connected to a terminal on the front of said carriage, a conductor and flexible lead between said terminal and cylinder, a wooden box on rear of said cylinder and a source of direct electric current.

2. Improved means for depositing a protective coating on metallic articles, including a colloidal solution or emulsion or fluxed bitumen and other ingredients in an aqueous medium from which said coating is deposited by electrolysis, an anode consisting of the positively charged water pipe to be coated, a cathode consisting of a negatively charged copper cylinder having at the ends travelling carriages of insulating material fitted with rubber discs or rings and leather washers, a supply of electrolyte sealed between said rings and washers, a hosepipe feeding said electrolyte to a tube running through the front carriage and emerging through the surface of the cathode cylinder, a waterproof cable connected to a terminal on front carriage, a conductor and flexible lead between said terminal and cathode cylinder, and a source of direct electric current.

3. Improved means for depositing a protective coating on metallic articles, including a colloidal solution or emulsion of fluxed bitumen and other ingredients in an aqueous medium from which said coating is deposited by electrolysis, an anode consisting of the positively charged water pipe to be coated, a cathode consisting of a negatively

charged metal plate curved to the inner surface of said water pipe, a box of insulating material holding said cathode plate and similarly curved, flexible rubber edging between said cathode plate and water pipe, a supply tube articulated to said box conveying a supply of electrolyte from a reservoir to the space between said cathode plate and the inner surface of the water pipe via a hosepipe and a tube emerging through the surface of the cathode plate and universally jointed by a ball and two cups between two trolleys, a travelling carriage formed of said trolleys which have wood wheels held against the top and bottom of the water pipe by two telescopic screwed struts on either side of said ball and cups and capable of being extended or contracted by two hand nuts to suit the diameter of the water pipe, a third telescopic screwed strut between the top of said supply tube and the water pipe controlled by hand nut and fitted with a friction pad to enable the cathode box and plate to be held against any portion of the water pipe by said ball and cups controlling radial movement and said trolleys controlling longitudinal movement, a waterproof cable connected to the cathode plate and a source of direct electric current.

In testimony whereof I have affixed my signature hereto this 23rd day of April 1930.

FREDERICK WILLIAM HAMMOND.

70

75

80

85

90

95

100

105

110

115

120

125

130